

Patented Feb. 6, 1923.

1,444,587

## UNITED STATES PATENT OFFICE.

LYMAN M. COOPER, OF DETROIT, MICHIGAN, ASSIGNOR OF ONE-HALF TO CHARLES E. WISNER, OF DETROIT, MICHIGAN.

COMPOSITION OF MATTER FOR MAKING BATTERY BOXES, COIL BOXES, AND OTHER SIMILAR ARTICLES.

No Drawing.

Application filed September 16, 1920. Serial No. 410,621.

106-93

*To all whom it may concern:*

Be it known that I, LYMAN M. COOPER, a citizen of the United States, residing at Detroit, county of Wayne, State of Michigan, have invented a certain new and useful Improvement in Composition of Matter for Making Battery Boxes, Coil Boxes, and Other Similar Articles; and declare the following to be a full, clear, and exact description of the same, such as will enable others skilled in the art to which it pertains to make and use the same, reference being had to the accompanying drawings, which form a part of this specification.

My invention relates to a new and useful composition of matter for use in the manufacture of battery boxes, coil boxes, steering wheel rims and other similar articles formerly made of wood. The principal object of the invention is to utilize waste products in the composition so that the completed article may be produced very cheaply and yet be of greater strength than a similar article made of wood. The composition consists of the following ingredients combined in substantially the proportions stated viz:

Leached wood ashes, air dried - 1 quart.  
Air slackened lime - 2 quarts.  
Linseed oil -  $\frac{1}{2}$  pint.  
A binder such as Portland cement, or calcium sulphate -  $\frac{1}{2}$  pint.  
A body such as sawdust, ground paper or ground leather -  $\frac{1}{2}$  bushel.

These ingredients are to be thoroughly mixed and the mass fed to a pug mill, the composition being forced from the pug mill into a mold of the desired form under pressure. The linseed oil is mixed with the material to lubricate the same while being passed through the pug mill, as the composition without the linseed oil is too dry to be forced therethrough. The material is pressed to approximately thirty tons per square inch in the mold thereby producing an article of great density and of rock like hardness which has about the lightness of wood.

The binder may be either Portland cement, calcium sulphate or the like, the object being to provide a material which will cement the several ingredients together and fill the small interstices in the body of the material making a close grained and dense article

when formed. The body may be either sawdust, ground paper, ground leather, or other waste material which may be utilized in the composition and which costs practically nothing and as the main body of the composition is of this material, the formed articles are made very cheaply and can be produced for considerably less cost than a similar article of wood and the formed article also having the added advantage of being formed in one homogeneous piece.

One of the most important features of this invention is that the articles after being pressed are ready for use and require no baking or drying as is customary with many compositions. Enough linseed oil must be added to allow the material to be fed through the pug mill but the linseed oil is not added in sufficient quantity to make the material plastic and dries out while the article is being formed or soon thereafter without changing the character of the composition. This composition is particularly satisfactory when formed into battery boxes, the acid from the battery having practically no effect on the composition and as the box with this composition is formed of one piece without seams it is not only acid proof but waterproof as well and will not crack, leak or come apart. This composition also proves very satisfactory for making coil boxes, the box being without seams and waterproof proves a very satisfactory protection for coils and other devices of like nature which require a waterproof container.

From the foregoing description it becomes evident that articles made of the ingredients mentioned may be more quickly and cheaply made than articles of similar nature formed of wood, the material at the same time being waterproof, of greater strength and greater hardness and density than wood.

Having thus fully described my composition what I claim and desire to secure by Letters Patent of the United States is—

1. The herein described composition of matter comprising leached wood ashes, air slaked lime, linseed oil, Portland cement and sawdust substantially as and for the purpose specified.
2. The herein described composition of matter for use in the manufacture of battery boxes, coil boxes, steering wheel rims and like articles comprising air dried and

leached wood ashes, air slaked lime, linseed, one-half bushel substantially as and for the 20 oil, a cementitious filler and a comminuted purpose specified. waste material as and for the purpose de- 5. The herein described composition of

5 3. The herein described composition of matter for use in the manufacture of battery boxes, coil boxes, steering wheel rims and other articles of like nature comprising leached wood ashes, air slaked lime, linseed oil, a cementitious filler and a comminuted fibrous material substantially as and for the purpose described.

10 4. The herein described composition of matter for use in the manufacture of battery boxes, coil boxes, steering wheel rims and other articles of like nature comprising air dried leached wood ashes 1 pt., air slaked lime—2 qts., linseed oil—one-half pint, Portland cement—one-half pint, and sawdust

15 matter for the manufacture of various articles usually made of wood which comprises a base of a comminuted fibrous material combined with which is leached wood ashes, air slaked lime, and a cementitious filler.

20 6. The herein described composition of matter for forcing into a mold by pressure to form various articles which comprises a base of fibrous material, leached wood ashes, air slaked lime, and a cementitious filler mixed with a self-drying oil to act as a lubricant in passing through the pressure applying and forming mechanism.

25 35 In testimony whereof, I sign this specification.

LYMAN M. COOPER.